# EUROPEAN PATENT SPECIFICATION

(11) **EP 0 084 138 B1**
(45) Date of publication and mention of the grant of the patent: **25.02.1987**
(21) Application number: 82111754.6
(22) Date of filing: 17.12.1982
(51) Int. Cl.: H01F 1/14, C22C 19/07

(54) **Near-zero magnetostrictive glassy metal alloys with high magnetic and thermal stability**
Metallegierungen mit Glasstruktur, einer Magnetostriktion in der Nähe von Null und hoher thermischer und magnetischer Stabilität
Alliages métalliques ayant une structure de verre, une magnétostriction de presque zéro et une grande stabilité magnétique et thermique

(30) Priority: 18.01.1982 US 340413
(43) Date of publication of application: 27.07.1983
(73) Proprietor: ALLIED CORPORATION, Morristown New Jersey 07960 (US)
(72) Inventor: Hasagawa, Ryusuke, Morristown New Jersey 07960 (US)
(74) Representative: Weber, Dieter, Dr.

## Description

### Background of the invention

### 1. Field of the invention

This invention relates to glassy metal alloys with near-zero magnetostriction, high magnetic and thermal stability and excellent soft magnetic properties.

### 2. Description of the prior art

Saturation magnetostriction AS is related to the fractional change in length Δl/l that occurs in a magnetic material on going from the demagnetized to the saturated, ferromagnetic state. The value of magnetostriction, a dimensionless quantity, is often given in units of microstrains (i.e., a microstrain is a fractional change in length of one part per million).

Ferromagnetic alloys of low magnetostriction are desirable for several interrelated reasons:
1. Soft magnetic properties (low coercivity, high permeability) are generally obtained when both the saturation magnetostriction Às and the magnetocrystalline anisotropy K approach zero. Therefore, given the same anisotropy, alloys of lower magnetostriction will show lower dc coercivities and higher permeabilities. Such alloys are suitable for various soft magnetic applications.
2. Magnetic properties of such zero magnetostrictive materials are insensitive to mechanical strains. When this is the case, there is little need for stress-relief annealing after winding, punching or other physical handling needed to form a device from such material. In contrast, magnetic properties of stress-sensitive materials, such as the crystalline alloys, are seriously degraded by such cold working and such materials must be carefully annealed.
3. The low dc coercivity of zero magnetostrictive materials carries over to ac operating conditions where again low coercivity and high permeability are realized (provided the magnetocrystalline anisotropy is not too large and the resistivity not too small). Also because energy is not lost to mechanical vibrations when the saturation magnetostriction is zero, the core loss of zero magnetostrictive materials can be quite low. Thus, zero magnetostrictive magnetic alloys (of moderate or low magnetocrystalline anisotropy) are useful where low loss and high ac permeability are required. Such applications include a variety of tape-wound and laminated core devices, such as power transformers, signal transformers, magnetic recording heads and the like.
4. Finally, electromagnetic devices containing zero magnetostrictive materials generate no acoustic noise under AC excitation. While this is the reason for the lower core loss mentioned above, it is also a desirable characteristic in itself because it eliminates the hum inherent in many electromagnetic devices.

There are three well-known crystalline alloys of zero magnetostriction (in atom percent, unless otherwise indicated):
(1) Nickel-iron alloys containing approximately 80% nickel ("80 nickel permalloys");
(2) Cobalt-iron alloys containing approximately 90% cobalt; and
(3) Iron-silicon alloys containing approximately 6 wt.% silicon.

Also included in these categories are zero magnetostrictive alloys based on the binaries but with small additions of other elements such as molybdenum, copper or aluminum to provide specific property changes. These include, for example, 4% Mo, 79% Ni, 17% Fe (sold under the designation Moly Permalloy) for increased resistivity and permeability; permalloy plus varying amounts of copper (sold under the designation Mumetal) for magnetic softness and improved ductility; and 85 wt.% Fe, 9 wt.% Si, 6 wt.% AI (sold under the designation Sendust) for zero anisotropy.

The alloys included in category (1) are the most widely used of the three classes listed above because they combine zero magnetostriction with low anisotropy and are, therefore, extremely soft magnetically; that is they have a low coercivity, a high permeability and a low core loss. These permalloys are also relatively soft mechanically and their excellent magnetic properties, achieved by high temperature (above 1000°C) anneal, tend to be degraded by relatively mild mechanical shock.

Category (2) alloys such as those based on Co₉₀Fe₁₀ have a much higher saturation induction (Bₛ about 1.9 Tesla) than the permalloys. However, they also have a strong negative magnetocrystalline anisotropy, which prevents them from being good soft magnetic materials. For example, the initial permeability of CogₒFeₗₒ is only about 100 to 200.

Category (3) alloys such as Fe/6 wt% Si and the related ternary alloy Sendust (mentioned above) also show higher saturation inductions (B_{S} about 1.8 Tesla and 1.1 Tesla, respectively) than the permalloys. However these alloys are extremely brittle and have, therefore, found limited use in powder form only. Recently both Fe/6.5 wt.% Si [IEEE Trans. MAG-16, 728 (1980)] and Sendust alloys [IEEE Trans. MAG-15, 1149 (1970)] have been made relatively ductile by rapid solidification. However, compositional dependence of the magnetostriction is very strong in these materials, difficult precise tayloring of the alloy composition to achieve near-zero magnetostriction.

It is known that magnetocrystalline anisotropy is effectively eliminated in the glassy state. It is therefore, desirable to seek glassy metal alloys of zero magnetostriction. Such alloys might be found near the compositions listed above. Because of the presence of metalloids which tend to quench the magnetization by the transfer of charge to the transition-metal d-electron states, however, glassy metal alloys based on the 80 nickel permalloys are either non-magnetic at room temperature or have unacceptably low saturation inductions. For example, the glassy alloy Fe₄₀Ni₄₀P₁₄B₆ (the subscripts are in atom percent) has a saturation induction of about 0.8 Tesla, while the glassy alloy Ni₄₉Fe₂₉P₁₄B₆Si₂ has a saturation induction of about 0.46 Tesla and the glassy alloy Ni₈₀P₂₀ is non-magnetic. No glassy metal alloys having a saturation magnetostriction approximately equal to zero have yet been found near the iron-rich Sendust composition. A number of near-zero magnetostrictive glassy metal alloys based on the Co-Fe crystalline alloy mentioned above in (2) have been reported in the literature. These are, for example, Co₇₂Fe₃P₁₆B₆Al₃ (AIP Conference Proceedings, No. 24, pp. 745-746 (1975)) Co_{70.5}Fe_{4.5}Si₁₅B₁₀ (Vol. 14, Japanese Journal of Applied Physics, pp. 1077-1078 (1975)) Co_{31.2}Fe_{7.8}Ni_{39.0}B₁₄Si⁸ (proceedings of 3rd International Conference on Rapidly Quenched Metals, p. 183, (1979)] and Co₇₄Fe₆B₂₀ [IEEE Trans. MAG-12, 942 (1976)]. Table I lists some of the magnetic properties of these materials.

The saturation induction (Bₛ) of these alloys ranges between 0.6 and 1.2 Tesla. The glassy alloys with Bₛ close to 0.6 T show low coercivities and high permeabilities comparable to crystalline supermalloys. However, these alloys tend to be magnetically unstable at relatively low (150°C) temperatures. On the other hand, the glassy alloys with Bₛ-1.2 Tesla tend to have their ferromagnetic Curie temperatures (Of) near or above their first crystallization temperatures (T_{cl}). This makes heat-treatment of these materials very difficult to achieve desired soft magnetic properties because such annealing is most effective when carried out at temperatures near 6_{f}.

Clearly desirable are zero magnetostrictive glassy alloys with higher magnetic and thermal stability and a saturation induction as high as possible.

### Summary of the invention

In accordance with the invention, there is provided a magnetic alloy that is at least 70% glassy, and which has a near-zero magnetostriction, high magnetic and thermal stability and excellent soft magnetic properties. The glassy metal alloy has the composition CoₐFe_{b}NiₑMo_{d}BₑSi_{f}, where a ranges from about 58 to 70 atom percent, b ranges from about 2 to 7.5 atom percent, c ranges from about 0 to 8 atom percent, d ranges from about 1 to about 2 atom percent, e ranges from about 11 to 15 atom percent and f ranges from about 9 to 14 atom percent, with the proviso that the sum of a, b and c ranges from about 72 to 76 atom percent and the sum of e and f ranges from about 23 to 26 atom percent. The glassy alloy has a value of magnetostriction ranging from about -1 x10⁻⁶ to +1 x10⁻⁶ a saturation induction ranging from about 0.6 to 0.8 Tesla, a Curie temperature ranging from about 550 to 670K and a first crystallization temperature ranging from about 790 to 870 K.

### Detailed description of the invention

In accordance with the invention, there is provided a magnetic alloy that is at least 70% glassy and which has an outstanding combination of properties, including a near-zero magnetostriction, high magnetic and thermal stability and such soft magnetic properties as high permeability, low core loss and low coercivity. The glassy metal alloy has the composition CoₐFe_{b}Ni_{c}Mo_{d}BₑSi_{f}, where a ranges from about 58 to 70 atom percent, b ranges from about 2 to 7.5 atom percent, c ranges from about 0 to 8 atom percent and d ranges from about 1 to about 2 atom percent, e ranges from about 11 to 15 atom percent and f ranges from about 9 to 14 atom percent, with the proviso that the sum of a, b and c ranges from about 72 to 76 atom percent and the sum of e and f ranges from about 23 to 26 atom percent. The glassy alloy has a value of magnetostriction ranging from about -1x10⁻⁶ to +1x10⁻⁶ and a saturation induction ranging from about 0.6 to 0.8 Tesla, Curie Temperature, ranging from 550 to 670K and the first crystallization temperature ranging from about 790 to 870 K.

The purity of the above composition is that found in normal commercial practice. However, it will be appreciated that molybdenum in the alloys of the invention may be replaced by at least one other transition metal element, such as tungsten, niobium, tantalum, titanium, zirconium and hafnium, and up to about 2 atom percent of Si may be replaced by carbon, aluminum or germanium without significantly degrading the desirable magnetic properties of these glassy alloys.

Examples of essentially zero magnetostrictive glassy metal alloys of the invention include

These glassy alloys possess saturation induction between about 0.7 and 0.8 Tesla, Curie temperature between 600 and 670K, the first crystallization temperature of about 800K and excellent ductility. Some magnetic and thermal properties of these and some of other near-zero magnetostrictive glassy alloys of the present invention are listed in Table II. These may be compared with properties listed in Table I for previously-reported glassy metal alloys of zero magnetostriction.

The activation energy (Eₐ) for the reorientation of the magnetization is listed in Table III for some representative near-zero magnetostrictive glassy alloys. This table indicates that Si tends to increase Eₐ and also that Eₐ tends to be higher when Si/B ratio is close to 1. The higher values of Eₐ, indicating higher magnetic stability of the system, is desired. Combining these information based Table II and III, preferred Si content is between 9 and 14 atom percent when (Si+B) is between 23 and 26 atom percent.

The presence of Mo is to increase Tₑₗ and hence the thermal stability of the alloy system. The content of Mo beyond 2 atom percent, however, reduces the Curie temperature to a level lower than 550 K, which is undesirable in convention magnetic devices.

For some applications, it may be desirable or acceptable to use a material with a small positive or a small negative magnetostriction. Such near-zero magnetostrictive glassy metal alloys are obtained for a, b and c in the ranges of about 58 to 70, 2 to 7.5 and 0 to 8 atom percent respectively, with the provision that the sum of a, b and c ranges between 72 and 76 atom percent. The absolute value of saturation magnetostriction λₛ of these glassy metal alloys is less than about 1x10⁻⁶ (i.e., the saturation magnetostriction ranges from about -1 x10⁻⁶ to +1 x10⁻⁶, or -1 to +1 microstrains). The saturation induction of these glassy alloys ranges between about 0.6 and 0.8 Tesla.

Values of λₛ even closer to zero may be obtained for values of a, b and c ranging respectively from about 63 to 69, 3 to 6 and 0 to 6, with the provision that the sum of a, b and c ranges between about 72 and 76 atom percent. For such preferred compositions, |λₛ |is less than 0.5x10⁻⁶. Essentially zero values of magnetostriction are obtained for values of a, b and c ranging from about 64 to 68, 4 to 5 and 0 to 6 atom percent respectively with the provision that the sum of a, b and c ranges between about 72 and 76 atom percent and also when f is between 11 and 12 atom percent and (e+f) is close to 24 atom percent and, accordingly, such compositions are most preferred.

The glassy metal alloys of the invention are conveniently prepared by techniques readily available elsewhere; see, e.g., U.S. Patents 3,845,805, issued November 5,1974 and 3,856,513, issued December 24, 1974. In general, the glassy alloys, in the form of continuous ribbon, wire, etc., are rapidly quenched from a melt of the desired composition at a rate of at least about 10⁵ K/sec.

A metalloid content of boron, and silicon in the range of about 23 to 26 atom percent of the total alloy composition is sufficient for glass formation, with boron ranging from about 11 to 15 atom percent and silicon ranging from about 9 to about 14 atom percent. As noted hereinabove, a ratio Si/B close to 1 and a Si content ("f") between 11 and 12 atom percent are most favorable because they lead to higher stability and relative insensitiveness of the magnetostriction value (which is close to,zero) to the metalloid composition. For example, the rate of change of magnetostriction value with respect to silicon content, dAₛ/df, is close to zero for "f" between 11 and 12 atom percent while |dλₛ/df |is about 0.8x 10⁻⁶/at. %Si near f=1 0 or 13 atom percent when a=67.1, b=4.5, c=3.0 and d=1.5 atom percent. The quantity dλₛ/df becomes zero near f=12 atom percent and about 0.1 x 10⁻⁶/at. %Si near f=10 or 13 atom percent when a=67.8, b=3.7, c=3.0 and d=1.5 atom percent.

The small amount of Ni is relatively ineffective to alter the magnetostriction values in the present alloy system and Co:Fe ratios essentially determine the resultant magnetostriction values. Zero magnetostriction is realized for the Co:Fe ratio of about (14-16.5) to 1 in the present alloy system. In the prior art glassy metal alloys such as Co_{70.5}Fe_{4.5}B₁₀Si₁₅ and Co₇₄Fe₆B₂₀. the ratios are narrowly set at about 14 and 12 respectively. The above range of the Co:Fe ratio between about 14:1 to 16.5:1 and the tolerance of about ±0.5 atom percent near f=₁₁.5 atom percent to achieve λₛ=0 and dλₛ/df=0 are advantageous from materials synthesis standpoint.

Table IV gives ac core loss (L), exciting power (Pₑ) and permeability (p) at 0.1 Tesla induction and at 50 kHz of the near-zero magnetostrictive glassy alloys of the present invention annealed at different temperatures (Tₐ).

Table V shows the effects of the annealing temperature (Tₐ) and annealing field (H₁₁) applied along the circumferential direction of the toroidal samples on the dc coercivity (H_{c}) and remanence (Bᵣ), ac coercivity (H_{c}) and squareness ratio (Bᵣ/B₁), where B₁ is the induction at an applied field of 1 Oe at 50 kHz and µ at 50 kHz and 0.1 T induction for one of the zero magnetostrictive alloys of the present invention. Low coercivity and high squareness ratio close to 1 at high frequencies (e.g. 50 kHz) are desirable in some magnetic device applications such as switch-mode power supplies.

Table VI shows the effects of the annealing time (tₐ) on L, Pe and µ for one of the zero magnetostrictive alloys of the present invention.

The results set forth in Tables IV-VI above indicate that L=4 W/kg, Pe=7 Va/kg and µ=23 000 at 0.1 T and 50 kHz can be achieved for 25-30 µm thick zero magnetostrictive glassy alloys of the present invention. Compared with these values, a prior art crystalline nonmagnetostrictive supermalloy of the similar thickness (25 µm) gives L=8 W/kg, Pₑ=10 VA/kg and p=19 000 at 0.1 T and 50 kHz. It is clear that the properties of the nonmagnetostrictive glassy alloys of the present invention are superior to those of the crystalline supermalloys. Examples of amorphous alloys outside the scope of the invention are set forth in Table VII. The advantageous combination of properties provided by the alloys of the present invention cannot be achieved in the prior art nonmagnetostrictive glassy alloys with high saturation induction such as Co₇₄Fe₆B₂₀ because their Curie temperatures are higher than the first crystallization temperatures and the heat-treatment to improve their properties are not so effective as in those with lower saturation inductions. The above properties, achieved in the glassy alloys of the present invention, may be obtained in low induction glassy alloys of the prior art. However, these alloys of the prior art such as Co_{31.2}Fe_{7.8}Ni_{39.0}B₁₄si₈ tend to be magnetically unstable at relatively low temperature of about 150°C as pointed earlier.

Table VII shows the magnetic properties of some of the representative glassy alloys of the composition COₐFe_{b}Ni_{c}MO_{d}BₑSi_{f} in which at least one of a, b, c, d, e, and f is outside the composition range defined in the present invention. The table indicates that the alloys with at least one of the constituents outside the defined ranges exhibit at least one of the following undesirable properties: (i) The value of |λₛ is larger than 1 x 10⁻⁶, (ii) The Curie temperature (S_{f}) is higher than the crystallization temperature (T_{cl}), which makes the post-fabrication field annealing less effective and (iii) The Curie temperature and saturation induction (Bₛ) become too low to be practical.

The following examples are presented to provide a more complete understanding of the invention. The specific techniques, conditions, materials, proportions and reported data set forth to illustrate the principles and practice of the invention are exemplary and should not be construed as limiting the scope of the invention.

### Examples

### 1. Sample preparation

The glassy alloys listed in Tables II-VII were rapidly quenched (about 10⁶ K/sec) from the melt following the techniques taught by Chen and Polk in U.S. Patent 3,856,513. The resulting ribbons, typically 25 to 30 pm thick and 0.5 to 2.5 cm wide, were determined to be free of significant crystallinity by X-ray diffractometry (using CuK radiation) and scanning calorimetry. Ribbons of the glassy metal alloys were strong, shiny, hard and ductile.

### 2. Magnetic measurements

Continuous ribbons of the glassy metal alloys prepared in accordance with the procedure described in Example I were wound onto bobbins (3.8 cm O.D.) to form closed-magnetic-path toroidal samples. Each sample contained from 1 to 3 g of ribbon. Insulated primary and secondary windings (numbering at least 10 each) were applied to the toroids. These samples were used to obtain hysteresis loops (coercivity and remanence) and initial permeability with a commercial curve tracer and core loss (IEEE Standard 106-1972).

The saturation magnetization, Mₛ, of each sample, was measured with a commercial vibrating sample magnetometer (Princeton Applied Research). In this case, the ribbon was cut into several small squares (approximately 2 mmx2 mm). These were randomly oriented about their normal direction, their plane being parallel to the applied field (0 to 720 kA/m. The saturation induction Bₛ (=4nM_{S}D) was then calculated by using the measured mass density D.

The ferromagnetic Curie temperature (θ_{f}) was measured by inductance method and also monitored by differential scanning calorimetry, which was used primarily to determine the crystallization temperatures. The first or primary crystallization temperature (Tₑₗ) was used to compare the thermal stability of various glassy alloys of the present and prior art inventions.

Magnetic stability was determined from the reorientation kinetics of the magnetization, in accordance with the method described in Journal of Applied Physics, vol. 49, p. 6510 (1978), which method is incorporated herein by reference thereto.

Magnetostriction measurements employed metallic strain gauges (BLH Electronics), which were bonded (Eastman-910 Cement) between two short lengths of ribbon. The ribbon axis and gauge axis were parallel. The magnetostriction was determined as a function of applied field from the longitudinal strain in the parallel (Δl/l)₁₁ and perpendicular (Δl/l)₁ in-plain fields, according to the formula

Having thus described the invention in rather full detail, it will be understood that this detail need not be strictly adhered to but that further changes and modifications may suggest themselves to one skilled in the art.

## Claims

1. A magnetic alloy evidencing near-zero magnetostriction, characterized in that it is at least 70% glassy, having the formula CoₐFe_{b}NiₑMo_{d}BₑSi_{f} where a ranges from about 58 to 70 atom percent, b ranges from about 2 to 7.5 atom percent, c ranges from 0 to 8 atom percent, d ranges from about 1 to 2 atom percent, e ranges from about 11 to 15 atom percent and f ranges from about 9 to 14 atom percent with the proviso that the sum of a, b and c ranges from about 72 to 76 atom percent and the sum of e and f ranges from about 23 to 26 atom percent, said alloy having a value of magnetostriction between -1x10⁻⁶ and +1 x 10⁻⁶.

2. The magnetic alloy of claim 1 in which a ranges from about 63 to 69 atom percent, b ranges from about 3 to 6 atom percent and c ranges from about 0 to 6 atom percent.

3. The magnetic alloy of claim 1 in which a ranges from about 64 to 68 atom percent, b ranges from 4 to 5 atom percent and c ranges from 0 to 6 atom percent when f is between 11 and 12 atom percent and the sum of e and f is near 24 atom percent.

4. The magnetic alloy of claim 3 having the formula Co_{67.4}Fe_{4.1}Ni_{3.0}Mo_{1.5}B_{12.5}Si_{11.5}

5. The magnetic alloy of claim 3 having the formula CO_{67.1}Fe_{4.4}Ni_{3.0}Mo_{1.5}B_{12.5}Si_{11.5}

6. The magnetic alloy of claim 3 having the formula Co_{64.0}Fe_{4.5}Ni_{6.0}Mo_{1.5}B_{12.5}.Si_{11.5}

7. The magnetic alloy of claim 3 having the formula Co_{67.0}Fe_{4.5}Ni_{3.0}Mo_{1.5}B₁₂Si₁₂

8. The magnetic alloy of claim 3 having the formula Co_{77.0}Fe_{4.5}Ni_{3.0}Mo_{1.5}B₁₃Si₁₁.

9. The magnetic alloy of claim 3 having the formula Co_{67.5}Fe_{4.5}Ni_{3.0}Mo_{1.0}B₁₂Si₁₂

## Patentansprüche

1. Magnetische Legierung mit einer Magnetostriktion nahe Null, dadurch gekennzeichnet, daß sie zu wenigstens 70% glasartig ist und die Formel CoₐFe_{b}Ni_{c}Mo_{d}BₑSi_{f} hat, worin a im Bereich von etwa 58 bis 70 Atom-%, b im Bereich von etwa 2 bis 7,5 Atom-%, c im Bereich von 0 bis 8 Atom-% d im Bereich von etwa 1 bis 2 Atom-%, e im Bereich von etwa 11 bis 15 Atom-% und f im Bereich von etwa 9 bis 14 Atom-% liegen, wobei die Summe von a, b und c im Bereich von etwa 72 bis 76 Atom-% und die Summe von e und f im Bereich von etwa 23 bis 26 Atom-% liegen und wobei die Legierung einen Magnetostriktionswert zwischen -1 x 10⁻⁶ und +1 x 10⁻⁶ hat.

2. Magnetische Legierung nach Anspruch 1, in welcher a im Bereich von etwa 63 bis 69 Atom-%, b im Bereich von etwa 3 bis 6 Atom-% und c im Bereich von etwa 0 bis 6 Atom-% liegen.

3. Magnetische Legierung nach Anspruch 1, in welcher a im Bereich von etwa 64 bis 68 Atom-%, b im Bereich von 4 bis 5 Atom-% und c im Bereich von 0 bis 6 Atom-% liegen, wenn f zwischen 11 und 12 Atom-% liegt und die Summe von e und f nahe 24 Atom-% ist.

4. Magnetische Legierung nach Anspruch 3 mit der Formel Co_{67.,4}Fe_{4,1}Ni_{3,0}Mo_{1,5}B_{12,5}Si_{11,5}

5. Magnetische Legierung nach Anspruch 3 mit der Formel Co_{67,1}Fe_{4,4}Ni_{3,0}Mo_{1,5}B_{12,5}Si_{11,5}

6. Magnetische Legierung nach Anspruch 3 mit der Formel Co_{64,0}Fe_{4,5}Ni_{6,0}Mo_{1,5}B_{12,5}Si_{11,5}

7. Magnetische Legierung nach Anspruch 3 mit der Formel Co_{67,0}Fe_{4,5}Ni_{3,0}Mo_{1,5}B₁₂Si₁₂.

8. Magnetische Legierung nach Anspruch 3 mit der Formel C0_{67,0}Fe_{4,5}Ni_{3,0}Mo_{1,5}B₁₃Si₁₁.

9. Magnetische Legierung nach Anspruch 3 mit der Formel Co_{67,0}Fe_{4,5}Ni_{3,0}Mo_{1,0}B₁₂ZSi₁₂.

## Revendications

1. Un alliage magnétique faisant preuve d'une magnétostriction presque nulle caractérisé en ce qu'il est vitreux à au moins 70%, ayant la formule CoaFebNieModBeSif dans laquelle a est compris entre environ 58 et 70 pour cent en atomes, b est compris entre environ 2 et 7,5 pour cent en atomes, c est compris entre 0 et 8 pour cent en atomes, d est compris entre environ 1 et 2 pour cent en atomes, e est compris entre environ 11 et 15 pour cent en atomes et f est compris entre environ 9 et 14 pour cent en atomes, à condition que la somme de a, b et c soit comprise entre environ 72 et 76 pour cent en atomes et que la somme de e et f soit comprise entre environ 23 et 26 pour cent en atomes, ledit alliage ayant une valeur de magnétostriction comprise entre -.1 - 10-⁶ et +1 - 10⁻⁶.

2. L'alliage magnétique de la revendication 1 dans lequel a est compris entre environ 63 et 69 pour cent en atomes, b est compris entre environ 3 et 6 pour cent en atomes et c est compris entre environ 0 et 6 pour cent en atomes.

3. L'alliage magnétique de la revendication 1 dans lequel a est compris entre environ 64 et 68 pour cent en atomes, b est compris entre 4 et 5 pour cent en atomes et c est compris entre 0 et 6 pour cent en atomes lorsque f est compris entre 11 et 12 pour cent en atomes et la somme de e et f est proche de 24 pour cent en atomes.

4. L'alliage magnétique de la revendication 3 ayant la formule Co_{67,4}Fe_{4,1}Ni_{3,0}Mo_{1,5}B_{12,5}Si_{11,5}

5. L'alliage magnétique de la revendication 3 ayant la formule Co_{67,1}Fe_{4,4}Ni_{3,0}Mo_{1,5}B_{12,5}Si_{11,5}

6. L'alliage magnétique de la revendication 3 ayant la formule Co_{64,0}Fe_{4,5}Ni_{6,0}Mo_{1,5}B_{12,5}Si_{17,5}·

7. L'alliage magnétique de la revendication 3 ayant la formule Co_{67,0}Fe_{4,5}Ni_{3,0}Mo_{1,5}B₁₂Si₁₂.

8. L'alliage magnétique de la revendication 3 ayant la formule Co_{67,0}Fe_{4,5}Ni_{3,0}Mo_{1,5}B₁₃Si₁₁.

9. L'alliage magnétique de la revendication 3 ayant la formule Co_{67,5}Fe_{4,5}Ni_{3,0}Mo_{1,0}B₁₂Si₁₂.
